

April 10, 1928.

1,665,360

C. G. HAWLEY

REINFORCEMENT FOR WELDED SEAMS

Original Filed May 13, 1922



Fig. 1



Fig. 2



Fig. 3



Fig. 4



Fig. 5



Fig. 6



Fig. 7



Fig. 8

C. G. Hawley  
Inventor.

## UNITED STATES PATENT OFFICE.

CHARLES GILBERT HAWLEY, OF CLEVELAND, OHIO.

## REINFORCEMENT FOR WELDED SEAMS.

Application filed May 13, 1922, Serial No. 560,671. Renewed February 23, 1928.

My invention relates to the art of uniting the edges of metal sheets one with the other by means of autogenous welds. That is, through the agency of the fusing of said 5 edges and the progressive addition of a molten metal of much the same nature as the sheets to be united. As is well known, autogenous welded seams in boiler sheets and the like, while often developing a strength and 10 durability exceeding the strength of a riveted seam, in one or the other common forms, cannot be relied upon as a seam of constant running strength or of constant ductility or 15 shock resisting strength. In consequence, it is not the practice to use autogenously welded 20 seams in places where they are subjected to tensile strains or heavy shock stresses. The characteristic lacking is that of assured strength in proportion to the cross section of 25 the given weld and the materials employed in making it.

The object of my invention is so to reinforce welded seams as to render them dependable in all respects, and further, one 25 object of this invention is to provide a reenforced autogenous welded seam which, if need be, may safely be used in places which are directly exposed to firebox flames. My 30 invention will be found to be of particular importance in the art of making boilers, wherein the seams are subjected to heavy pressures and strains, but obviously is applicable throughout the metallurgical arts wherever welded seams require reinforcement.

The invention will be readily understood on reference to the accompanying drawings, in which Fig. 1 is a cross section of a metal tube or cylinder welded and reenforced in 40 accordance with this invention; Fig. 2 is a side view thereof; Fig. 3 is a vertical section of a boiler water wall or water leg presenting a reenforced welded seam; Fig. 4 is a side view thereof; Fig. 5 is a like view showing 45 the reenforcing weld completed and illustrating a different spacing of the stay-bolts; Fig. 6, is a horizontal section showing how the flanged together edges of a water wall may be welded and reenforced by my invention; Fig. 50 7 is a perspective view of the lower end of a Nicholson thermic siphon presenting a seam ready for reenforcement in the manner indicated in Figs. 6 and 8; Fig. 8 is a cross section of a thermic siphon neck or intake portion substantially on the line 8-8 of Fig. 7, showing how the reenforcement which I ap-

ply plays an advantageous part in the holding of the arch brick usually associated with thermic siphons in locomotive fireboxes. In each of the sectional figures there will be observed a V-weld, 2, which is made either by the electric or oxy-acetylene autogenous welding process. It is this welding which is to be reenforced in each case. For the reenforcement of the weld 2, I employ a sinuous 60 metal rod 3, preferably of rectangular cross section and of less width than height. This sinuous section is first conformed to the curved or flat surface of the united sheets (for comparison see Figs. 1 and 3) and is 65 laid flat against the naked surfaces of the sheets. The undulations or bends of the rod 3 are deep enough to reach far to one side and the other of the weld 2 so that naked surfaces 4 of the sheets are exposed in the bends. 70 Upon these surfaces and the inner surfaces 75 of the rod 3 I apply welding material by the autogenous process and thus build up abutments united with the rod and, obviously, situated on both sides of the weld 2. In this 80 manner the edges of the sheets, in addition to being united with the weld 2, are laced together by the sinuous rod 3.

Having secured the sinuous rod in the described relation, I then preferably proceed 85 with the addition of welding material until all of the outstanding surfaces of the rod are imbedded in welding material 5, as best shown in Fig. 5.

It is apparent that as the engaging surfaces of the abutted sheets and the sinuous rod respectively, are not welded together, there must necessarily be a thin air filled space or gap between them, conforming to the bends and connecting portions of the 90 sinuous rod. However such a gap is so 95 small relative to one formed by a straight lapping strip having the same lateral reach from one side to the other of the weld 2 as in no appreciable manner to interfere with the 100 transmission of heat. It will be understood that if the rod were of greater width the extent of the air gap would be increased.

Further, the mass of welding material 5 wherein the rod is imbedded and by which 105 it is united to the sheets insures the rapid conduction of heat through the plates or sheets and there is therefore little, if any, tendency for the reenforced weld to burn away even when exposed to fire of great intensity. The rod 3 in each case may be the same or of better material than that compos-

ing the sheets which are welded together, and, as will be apparent, the whole strength of the laced or reenforcing bar or rod is positively added to the strength of the automatically welded seam.

A unique use of this seam reenforcement which I claim is depicted in Fig. 8. In using thermic siphons in locomotive fireboxes it is necessary that they shall serve to support the fire brick arch therein. The tubular neck portion S of the siphon S' is of such size as to afford a rather poor support or abutment for the brick, and it has been necessary to apply studs on the sides thereof to prevent the brick from falling off. A reenforced seam S'' of the kind above described is made of the same width as the body of the siphon S' and by forming a laced portion upon the top of the neck provides a pair of ideal brick abutments S<sup>3</sup> thereon.

These reenforced welds have a greater strength than the initial sheets and a greater and more reliable strength than a riveted seam and may be used upon any part of a boiler or the like notwithstanding the excessive pressures and strains incident to such use.

Having thus described my invention, I claim as new and desire to secure by Letters

30 Patent:

1. In combination with a butt welded seam connecting marginal plate portions, a

sinuous bar disposed in flat engagement with parts of said plate portions and crossing and recrossing said seam and being embedded in welding material upon said marginal plate portions and said seam.

2. In combination with a butt welded seam connecting marginal plate portions, a sinuous bar crossing and recrossing said seam and having a flat surface disposed in close engagement with parts of said plate portions and seam respectively, and lines of welding disposed at the sides of and following the contour of said bar for securing the same to said marginal plate portions and seam respectively.

3. In combination with a butt welded seam connecting marginal plate portions, a bar of sinuous form including laterally spaced reverse curved parts and other parts connecting the same, said bar having a flat bottom surface and being engaged with parts of said plate portions and seam with said curved parts spaced a considerable distance beyond the seam which is crossed and recrossed by said parts connecting said laterally spaced curved parts of the bar, and lines of welding following the sides of said sinuous bar and securing the same to said plate portions and seam.

In testimony whereof, I have hereunto set

my hand this 6th day of May, 1922.

CHARLES GILBERT HAWLEY.